

## UNITED STATES PATENT OFFICE

2,474,034

## BLEACHING POPLAR GROUNDWOOD

Kenneth A. Craig, Appleton, Wis., assignor to  
Paper Patents Company, a corporation of Wis-  
consin

No Drawing. Application December 4, 1946,  
Serial No. 713,917

2 Claims. (Cl. 8—106)

1

The present invention relates to poplar groundwood and more particularly to the bleaching of poplar groundwood for use in the paper industry.

Illustrative species of woods known in the trade as "poplar" are *Populus*: *tremuloides*, *balsamifera*, *grandidentata*, *deltoidea*, *heterophylla* and *trichocarpa*. These poplar woods sometimes referred to as aspen, balsam poplar, large tooth aspen, cottonwood, swamp and black cottonwood respectively, have not been used as a source of mechanical or groundwood pulp for high grade book paper furnishes and the like because of the high percentage of decay or rot in standing trees. This decay, a characteristic of every kind of poplar and known as sap and heart rot or "brown rot," produces dirty and specky groundwood pulp making the same unfit for use in high grade furnishes or in the manufacture of white or light colored papers.

The rot is caused by fungi such as false tinder fungus (*Fomes igniarius*), butt-rot fungus (*Fomes applanatus*), etc. and as it is a general rule attacks the heart or center of the trees it is difficult if not impossible to ascertain contamination or decay by an inspection of the standing trees. This property of the fungi makes the use of rot-free poplar economically impractical due to high cost of cutting, examination thereafter with sorting out of wood containing rot, etc. In view of this coupled with the danger of spoiling or rendering unusable a batch of groundwood by failure to discover the presence after cutting of even a very small amount of rot, it has been found commercially impractical to use poplar as a source for high grade mechanical pulps. This presented the paper industry with an acute problem, for poplar, a wood available in large amounts, yields a white groundwood fiber of the type desired.

The principal object of the present invention is to provide a process for producing improved poplar groundwood adaptable for use in high grade furnishes in the paper industry.

Other objects will be apparent as the description proceeds hereinafter.

At the start of the investigation leading to the present invention it was discovered that the fungi rots of the poplar were complex compositions having peculiar properties. Some chemicals such as sulphur dioxide ( $SO_2$ ), although capable of bleaching ordinary woods, were found to have substantially no bleaching effect on fungi rot.

After a prolonged research investigation I discovered that poplar groundwood containing the fungi or brown rot may be rendered usable in

5 high grade furnishes by subjecting the groundwood to an initial alkaline hypochlorite bleaching treatment followed by a subsequent acidifying or acid treatment, both treatments being carried out within the critical limits set forth below. The following examples will serve to illustrate the present invention.

*General example*

- 10 Poplar groundwood slurry of about 2-40 per cent O. D. (oven dry) consistency and at a temperature of about 25°-50° C. is treated with an aqueous solution of an alkaline material such as sodium hydroxide, sodium carbonate and calcium hydroxide, and a hypochlorite such as an alkaline earth or alkali metal salt, e. g. calcium hypochlorite. Sufficient of the hypochlorite is used to provide about 7-15 per cent of available chlorine on the O. D. groundwood basis. The hypochlorite is 15 usually mixed with the groundwood in a relatively short time although the hypochlorite may be added intermittently or more slowly thereby requiring a longer time for the complete addition. A portion of the alkaline constituent may be 20 mixed with the hypochlorite and the remainder added separately or the alkaline constituent may be added simultaneously with and continuously or intermittently after the hypochlorite. Sufficient quantities of the alkaline material (sodium 25 hydroxide is preferred as it yields the best results) are used to provide and maintain a pH of about 9-11 during the bleaching reaction.
- It has been found necessary to maintain the pH within the above range during the major portion of the bleaching process. A more alkaline condition results in a discoloration of the pulp which bleaches with greater difficulty and a pH value appreciably below 9.0 causes the groundwood pulp to acquire a reddish coloration resembling chlorination, and results in the consumption of more chlorine to obtain the same result. The bleaching action is allowed to proceed until the available chlorine is essentially consumed which requires from 10 minutes to several 30 hours depending upon the consistency, temperature, pH, per cent available chlorine used, etc., and the mixture is subjected to intermittent or preferably continuous agitation during the bleaching action.
- 40 After the hypochlorite treatment and the available chlorine is substantially consumed, a necessary condition in order to prevent the formation of the reddish coloration, the groundwood mixture is acidified, i. e. the pH is lowered or made 45 acid, by addition of an acidic material to a pH of 50

4.0-7.0 with a pH of 5.0-5.5 being preferred. The acidic materials include acid bisulfites and mineral acids as well as organic acids, sulfurous acid and alum being two preferred materials. The mixture after acidification may or may not be washed prior to using in paper furnish in accordance with the standard practices in the paper art.

*Example*

According to the above procedure, an aqueous slurry of rot infected groundwood at about 5 per cent consistency was placed in a tank and treated at a temperature of about 40° C. with an aqueous solution of calcium hypochlorite. The available chlorine, based on the groundwood, was about 10.7 per cent. This is in accordance with the preferred procedure employing approximately 10 per cent available chlorine based on the groundwood. Sodium hydroxide was added continuously to the groundwood-calcium hypochlorite mixture so as to maintain the reaction mixture at a pH of about 10.5. The treatment was continued until the available chlorine was consumed, which took about 20-30 minutes. The alkaline reaction mixture was then pumped into a storage chest from whence it was continuously pumped into an acidification tank and mixed with sufficient sulphurous acid to bring the pH of the slurry down to about 5.0-5.5.

In one month's commercial operation of the above process, about 1,236 tons (air-dry basis) of poplar groundwood contaminated by fungi or brown rot was treated using about 378.2 tons of calcium hypochlorite (containing 35 per cent available chlorine) and about 58.7 tons of sodium hydroxide. From this operation 1,198 tons (air-dry basis) of washed, bleached groundwood pulp was obtained. This data shows a loss of about 38 tons, which means a yield of about 97 per cent.

Investigations show that poplar groundwood pulp bleached in accordance with the preferred conditions of the present invention has a brightness of 74-75 as measured on the General Electric Reflectance Meter and that the bleached pulp even when the original wood contains relatively large amounts of fungi rot is adaptable for use in high grade news and book paper furnishes. Investigations also show that the fiber strength of poplar groundwood is not deleteriously affected by the bleaching treatment of the present invention. Investigations further show that very small loss (less than 1 per cent in small operations and about 3 per cent in large scale commercial operations) is experienced as a result of the chemical treatment of the poplar groundwood in accordance with the present invention.

The poplar groundwood treated in accordance with the present invention in addition has been found particularly adaptable for use in paper with alkaline fillers or coating pigments such as calcium carbonate. While no filler is formed when sodium hydroxide is employed as the alkaline material, it will be noted that calcium carbonate filler may be formed in situ by employing sodium carbonate as the alkaline material in

combination with calcium hypochlorite. Alkaline fillers or pigments, due to discoloration, are not as a general rule adaptable for use with groundwood or mechanical pulps containing all the constituents of the original wood.

Large scale operations show the hypochlorite bleaching treatment of the present invention to be economically and commercially practical. The loss during the chemical treatment of poplar is unexpectedly low and commercial operations show that the process of the present invention provides the art with a satisfactory means for utilizing poplar groundwood in high grade paper furnishes.

This application is a continuation in part of my co-pending application, Serial No. 388,803 filed April 16, 1941, now abandoned.

I claim:

1. In the paper art, the process of treating poplar groundwood contaminated with fungi rot which comprises subjecting the contaminated groundwood to the action of an alkaline hypochlorite solution having a pH value of about 9-11 and a temperature of about 25°-50° C., sufficient hypochlorite being present to provide about 7-15 per cent available chlorine based on the groundwood, and then acidifying said solution after the consumption of the available chlorine.
2. In the paper art, the process of treating poplar groundwood contaminated with fungi rot, which comprises subjecting the contaminated groundwood to the bleaching action of an aqueous sodium hydroxide-calcium hypochlorite solution at a temperature of about 25°-50° C., said solution having a pH value about 9-11 and containing sufficient hypochlorite to provide about 7-15 per cent available chlorine based on the groundwood, and after the consumption of the available chlorine subjecting said groundwood to an acid treatment by addition of sulphurous acid to said solution.

KENNETH A. CRAIG.

REFERENCES CITED

The following references are of record in the file of this patent:

UNITED STATES PATENTS

| 50 | Number    | Name            | Date           |
|----|-----------|-----------------|----------------|
|    | 11,786    | Horsford        | Oct. 10, 1854  |
|    | 348,165   | Just et al.     | Aug. 24, 1886  |
|    | 481,414   | Myrick          | Aug. 23, 1892  |
| 55 | 1,468,693 | Baker           | Sept. 25, 1923 |
|    | 1,645,061 | Kress           | Oct. 11, 1927  |
|    | 2,020,437 | Smith           | Nov. 12, 1935  |
|    | 2,046,382 | Hirschkind      | July 7, 1936   |
|    | 2,187,016 | Craig           | Jan. 16, 1940  |
|    | 2,359,891 | Brallier et al. | Oct. 10, 1944  |

60 FOREIGN PATENTS

| Number  | Country       | Date          |
|---------|---------------|---------------|
| 298,333 | Great Britain | Oct. 11, 1928 |

65 OTHER REFERENCES

Munro—"The Grinding of Wood Infected by Fungi," Paper Industry, July 1920, page 564.